

Sept. 11, 1956

H. L. BEDELL ET AL

2,762,757

ASPHALT AND METHOD OF PRODUCING THE SAME

Filed Dec. 17, 1952



INVENTORS

Harold L. Bedell  
Walter C. Fry  
Roy T. Evans

BY

*Robert D. Lynn*

AGENT

1

2,762,757

## ASPHALT AND METHOD OF PRODUCING THE SAME

Harold L. Bedell, Roy T. Evans, and Walter C. Fry, Augusta, Kans., assignors to Socony Mobil Oil Company, Inc., a corporation of New York

Application December 17, 1952, Serial No. 326,506

4 Claims. (Cl. 196—74)

This invention has to do with asphalts and with a method for producing the same.

In recent years, asphalts possessing a particular combination of properties have been developed for many specialty applications, such as paper saturants in the paper art. These asphalts are characterized by a low viscosity with a large change in viscosity on heating, good thermal stability, and dryness at any given point. They are generally referred to as "cracked" or "synthetic" asphalts inasmuch as they are prepared by thermal cracking of gas oil stocks.

So advantageous are these "cracked" or "synthetic" asphalts that demand has far exceeded supply. To meet this demand, attention has been focused upon other more available hydrocarbon stocks as replacements for the stocks from which synthetic asphalts are usually produced. However, such other stocks as are in supply have not responded to the same thermal cracking operations to yield the desired products.

It is an object of this invention, therefore, to provide a new method for preparing asphalts having the properties of "cracked" or "synthetic" asphalts. It is also an object to provide a method for preparing the desired asphalts from hydrocarbon stocks of conventional residual asphalts, which hydrocarbon stocks are in good supply and are relatively inexpensive. Other objects and advantages of the invention will be apparent from the following description.

It has now been found that outstanding asphalts, comparable to "cracked" or "synthetic" asphalts, can be prepared from straight run asphalts by a particular sequence of operations. A straight run asphalt is blended with a cyclic gas oil of low aniline number, the blend is then subjected to a heat treatment or cracking operation and the product thus obtained is thereafter reduced to provide the desired asphalt product.

As indicated above, the particular sequence of operations which makes possible production of the desired asphalts of this invention is:

- (1) Blending a straight run asphalt with a regulated quantity of a cyclic gas oil of a "refractory" nature,
- (2) Heat treating or cracking the blend, formed in (1) to a desired asphalt quality, and
- (3) Reducing the heat treated or cracked blend to an asphalt of desired character.

The charge stocks used herein are, as indicated above, straight run asphalts and cyclic gas oils. The asphalt charge can be, broadly, any petroleum residuum or flux which remains following the separation of the volatile oils from the crude. The separation of these volatile oils can be accomplished by means of vacuum distillation, steam distillation or by propane deasphalting. For ex-

2

ample, residua from Pennsylvanian, Mid-Continental, Californian, Mid-East, Near East, Venezuelan, etc. crudes can be used. Or, in other words, residua from paraffinic, naphthenic, aromatic, high-sulfur stocks, etc. are suitable. It will be recognized, of course, that differences in charge stocks are reflected in differences in character of the final products contemplated herein. The following analyses are typical of the asphalt charge stocks found to be advantageous:

|    |                                 |           |
|----|---------------------------------|-----------|
| 10 | Soft point, ring and ball, ° F. | 130-150   |
|    | Specific gravity                | 1.01-1.03 |
|    | Penetration:                    |           |
|    | @ 32° F., 200 g., 60 secs       | 5-13      |
|    | @ 77° F., 100 g., 5 secs        | 20-50     |
|    | @ 115° F., 50 g., 5 secs        | 70-175    |
|    | Viscosity, Furol, secs.:        |           |
|    | @ 275° F.                       | 300-800   |
| 20 | @ 300° F.                       | 150-400   |

The gas oils used herein are cyclic in character, and are resistant to thermal cracking. Gas oils of this character are well known in the art as "refractory stocks." 25 They are generally prepared by catalytic or thermal cracking processes such as typified by the Thermoform Catalytic Cracking (TCC) process or thermal cracking processes. Representative cyclic gas oils are the following oils designated A and B:

|    |                                    | Oil A | Oil B |
|----|------------------------------------|-------|-------|
| 35 | Aromatics, Percent by wt.          | 25    |       |
|    | Unsaturates, Percent by wt.        | 59    |       |
|    | API Gravity                        | 7.0   | 22.3  |
|    | Aniline Number                     | 90    | 174   |
|    | Four Point                         | +80   | +85   |
|    | Flash, ° F.                        | 380   | 365   |
|    | Distillation, ° F.:                |       |       |
|    | IBP                                | 550   | 503   |
|    | 20%                                | 710   | 650   |
|    | 50%                                | 780   | 706   |
|    | 90%                                | 890   | 737   |
|    | 95%                                | 910   | 810   |
|    | Sulfur                             | 1.4   |       |
|    | Hydrogen to Carbon Ratio           | 9.4   | 7.5   |
|    | Kinematic Viscosity (centistokes): |       |       |
| 40 | @ 100° F.                          | 117.0 | 16.15 |
|    | @ 210° F.                          | 11.4  | 3.33  |

Oils A and B are shown as representative charge stocks. Oil A is an oil which has been converted in the process contemplated herein, to asphalts of very desirable properties for uses that demand a synthetic type asphalt. Oil B is an oil which has been converted herein to asphalts having satisfactory properties, the properties falling between those characteristic of a straight run asphalt and those of a synthetic asphalt. That is, asphalts produced from oil B are not so desirable as asphalts produced from oil A. It will be noted that oil B is less cyclic or aromatic in character than is oil A. It is concluded, therefore, that oils having less aromaticity (indicated by higher aniline numbers) than oil B are not suitable in the process of this invention.

The proportions of the asphalt charge and gas oil can be varied considerably within certain limits, depending upon the source of the asphalt charge and upon the refractory nature of the gas oil. In general, however, from about 10 to 40 per cent by weight is made up of the asphalt charge, with the balance gas oil. By way of illustration, a vacuum reduced straight run asphalt, having a

ring and ball soft point of 130-150° F., is used advantageously in amounts of 20-30 per cent, by weight, with 80-70 per cent of a gas oil such as the oil identified as "A," hereinabove.

As contemplated herein, heat treatment or cracking of the asphalt gas oil blend is conducted in the liquid phase under selected conditions of temperature and time. In general, temperatures of the order of 875 to 900° F. with time intervals of five to three minutes are used; that is, the lower temperatures generally require the longer time intervals. Under such conditions as the foregoing, the resulting asphalt becomes in nature similar to the synthetic asphalts.

Following the asphalt conversion or cracking operation, the product obtained hereby is reduced at a maximum temperature of about 800° F. This is advantageously accomplished by distillation, with vacuum or with steam. For example, the heat modified or cracked product may be separated into overhead distillate and asphalt residue by vacuum or steam distillation.

The conditions of reduction to asphalt do not have any effect on the basic properties of the asphalt. The asphalt properties are fixed by the previous heat treatment and the composition of the blend treated. The reduction is merely a means of separating out the asphalt from the other products of the heat treated blend.

A typical operation contemplated herein is illustrated by the flow sheet shown in the attached drawing. A blend of cyclic gas oil and asphalt charge is pumped from charge blend tank 1 through line 2, by means of pump 3, to preheater 4, through line 5.

The blend is passed through line 6, positioned in the central portion of preheater 4, where the oil is heated to about 750° F.

The heated blend is removed from the preheater 4 through line 7 and is led into the upper portion of a cracking furnace 8. The blend flows through the furnace (8) via line 9, and leaves the furnace at about 850-900° F. via line 10. The heat treated or cracked product in line 10 is then led through the pressure relief valve (11). From the pressure relief valve, the product goes through line 10 to conventional vacuum distillation equipment and is thereby separated into overhead distillate and asphalt bottoms.

Oils A and B were each blended with twenty per cent by weight of 140 soft point, straight run asphalt (C) and heat treated as indicated below:

|                                      | Oil A, 80%, with 20% Asphalt C | Oil B, 80%, with 20% Asphalt C |
|--------------------------------------|--------------------------------|--------------------------------|
| Furnace Outlet Temp., °F             | 890                            | 891                            |
| Soaking Factor                       | 0.188                          | 0.207                          |
| Analysis of Resulting Asphalt:       |                                |                                |
| Soft Point, °F                       | 143                            | 143                            |
| Sp. Gr. 77/77                        | 1.1214                         | 1.0889                         |
| Penetration:                         |                                |                                |
| 100-5-77                             | 9                              | 15                             |
| 100-5-110                            | 480                            | 590                            |
| Flash                                | 90-95                          | 75                             |
| Xylene Equivalent                    | 0-196+                         | 16-182                         |
| Ductility                            | 99.84                          | 99.88                          |
| Solubility in CCl <sub>4</sub>       |                                |                                |
| Viscosity (Centipoises):             |                                |                                |
| @350° F                              | 48                             | 84                             |
| @325° F                              | 85                             | 150                            |
| @300° F                              | 173                            | 284                            |
| @275° F                              | 375                            | 640                            |
| @250° F                              | 918                            | 1555                           |
| Viscosity Temperature Susceptibility | 0.946                          | 0.845                          |

Analysis of the straight run asphalt (C) before processing is recited below:

|                      |       |
|----------------------|-------|
| Soft point, °F       | 144   |
| Sp. Gr. 77/77        | 1.017 |
| Penetration 100-5-77 | 28    |
| Xylene equivalent    | 0     |
| Ductility 5 cm. @ 77 | 47-56 |

Viscosity (centipoises):

|          |      |
|----------|------|
| @ 350° F | 176  |
| @ 325° F | 310  |
| @ 300° F | 584  |
| @ 275° F | 1210 |
| @ 250° F | 2640 |

Viscosity temperature susceptibility 0.733

From the foregoing results and analysis, it will be noted that the charge of Oil A and straight run asphalt (C) is converted to an asphalt having properties corresponding to those of synthetic asphalts. The charge of Oil B and (C) is also converted to a modified asphalt. Again, it is emphasized that Oil B has a higher aniline number than Oil A, indicative of lesser aromaticity, and that the greater the aromatic character of the charge oil the more desirable is the final product.

Tabulated below are data obtained by treating two blends of Oil A and the straight run asphalt (C). The blends were heat treated under similar conditions and then reduced to asphalts of the 140 soft point range.

|                                      | 66.6% Oil A with 33.4% Asphalt C | 80% Oil A with 20% Asphalt C |
|--------------------------------------|----------------------------------|------------------------------|
| Furnace Outlet Temp., °F             | 875                              | 890                          |
| Soaking Factor                       | 0.15                             | 0.19                         |
| Analysis of Resulting Asphalt:       |                                  |                              |
| Sp. Gr. 77/77                        | 1.0763                           | 1.1214                       |
| Soft Point, °F                       | 142                              | 143                          |
| Flash, CO <sub>2</sub> , °F          | 530                              | 480                          |
| Penetration, 100-5-77                | 18                               | 9                            |
| Xylene Equivalent                    | 75-80                            | 90-95                        |
| Solubility CCl <sub>4</sub>          | 99.76                            | 98.84                        |
| Ductility                            | 61-67                            | 0-196+                       |
| Viscosity (centipoises):             |                                  |                              |
| @350° F                              | 66                               | 48                           |
| @325° F                              | 127                              | 55                           |
| @300° F                              | 216                              | 173                          |
| @275° F                              | 355                              | 375                          |
| @250° F                              | 1.010                            | 918                          |
| Viscosity Temperature Susceptibility | 0.841                            | 0.946                        |

The data tabulated immediately above reveal that the greater the quantity of cyclic gas oil charge, the greater the modification of the asphalt charge. However, there is a practical or economical limit to the quantity of gas oil which can be used in the charge, since the larger quantity of the gas oil increases the quantity of oil processed for the amount of modified asphalt produced.

Additional data is presented below in order to demonstrate the influence of heat treating or cracking conditions upon the final product. In each of the Runs given below, a blend comprising two parts of Oil A and one part of the straight run asphalt (C) was used.

| Run No.                              | 1      | 2      | 3      |
|--------------------------------------|--------|--------|--------|
| Processing Temp., °F                 | 815    | 875    | 905    |
| Soaking Factor                       | 0.0171 | 0.1514 | 0.3192 |
| Analysis of Resulting Asphalt:       |        |        |        |
| Soft Point, °F                       | 144    | 142    | 144    |
| Penetration, 100-5-77                | 25     | 18     | 13     |
| Flash, °F                            | 545    | 530    | 535    |
| Solubility CCl <sub>4</sub>          | 99.74  | 99.76  | 95.75  |
| Xylene Equivalent                    | 0-5    | 75-80  | 100+   |
| Ductility, 5 cm. @ 77                | 42-45  | 61-67  | 38-42  |
| S. E. Viscosity (C. P.):             |        |        |        |
| @400° F                              | 60     |        |        |
| @375° F                              | 98     |        |        |
| @350° F                              | 157    | 66     | 68     |
| @325° F                              | 275    | 127    | 108    |
| @300° F                              | 570    | 216    | 215    |
| @275° F                              |        | 355    | 700    |
| @250° F                              |        | 1,010  | 1,200  |
| Viscosity Temperature Susceptibility | 0.683  | 0.841  | 0.876  |
| Soft Point-Penetration Index         | -0.05  | -1.8   | -1.2   |
| Ductility Coefficient                | 3.42   | 4.0    | 4.22   |

From the results directly above, it is concluded that the soaking factor maintained in Run 1 is too mild to provide the desired result. The character of asphalt

product of Run 1 is only slightly different from the character of the straight run asphalt of the charge. The asphalt product of Run 2 has desirable properties, thereby indicating that the heat treatment was suitable. In Run 3, the conditions of operation are approaching the upper limit of severity inasmuch as the "Solubility CCl<sub>4</sub>" value indicates the presence of some coke-like material in the product.

In general, the products of this invention are characterized by the following properties:

|                                                    | Broad Range  | Preferred Range |
|----------------------------------------------------|--------------|-----------------|
| Soft Point, °F                                     | 120 to 170   | 130 to 150      |
| Sp. Gr., 77/77                                     | 1.04 to 1.20 | 1.08 to 1.16    |
| Penetration: 100 gms., 5 secs., 77° F.             | 0 to 35      | 5 to 20         |
| Xylene Equivalent                                  | 5 to 100+    | 60 to 100+      |
| Ductility @ 77° F.                                 | 0 to 100+    | 40 to 100+      |
| Solubility (CCl <sub>4</sub> )                     | 95.0 to 100  | 98.0 to 100     |
| Viscosity in Centipoises:                          |              |                 |
| @ 250° F.                                          | 600 to 1,000 |                 |
| @ 275° F.                                          | 200 to 400   |                 |
| @ 300° F.                                          | 100 to 200   |                 |
| @ 325° F.                                          | 50 to 100    |                 |
| @ 350° F.                                          | 30 to 50     |                 |
| Viscosity Temperature Susceptibility (250-350° F.) | 0.78 to 1.2  | 0.9 to 1.0      |

Typical uses to which the asphalt products of this invention can be put are the following: water-proofing of paper; size or coating for insulation board; saturant for panel and molding boards made from Kraft paper; emulsions for briquetting of coal; preparation of molding compounds; saturant or binder for rock wool or fiber glass; for compounding with resins, such as vinsol resins.

The gas oils recovered with the asphalt products are

also of considerable value. They are used as rubber softeners, saturants for felt and papers, resin plasticizers, etc. and fuels.

We claim:

1. The process for producing a synthetic modified asphalt, characterized by a low viscosity with a large change in viscosity on heating, and good thermal stability which comprises: heat treating at a temperature from about 850° F. to about 900° F. for a period of time from about five minutes to about three minutes, a blend of a straight run asphalt and of a cyclic gas oil, said blend comprising from about ten to about forty weight per cent of said straight run asphalt; and reducing the product obtained by said heat treatment, whereby said modified asphalt is obtained.
15. 2. The process defined by claim 1 wherein the cyclic gas oil contains about twenty-five per cent by weight of aromatics.
3. The process defined by claim 1 wherein the straight run asphalt has a ring and ball soft point (° F.) from about 130 to about 150.
20. 4. The process defined by claim 1 wherein a soaking factor from about 0.1 to about 0.35 is maintained in said heat treatment.

25

References Cited in the file of this patent

UNITED STATES PATENTS

- |           |          |               |
|-----------|----------|---------------|
| 1,881,753 | Loebel   | Oct. 11, 1932 |
| 2,542,608 | Winkler  | Feb. 20, 1951 |
| 2,658,857 | Roediger | Nov. 10, 1953 |
| 2,662,051 | Pelzer   | Dec. 8, 1953  |